

# United States Patent

Chapman et al.

[15] 3,649,266

[45] Mar. 14, 1972

[54] **MAGENTA DYE DEVELOPER AND TRANSFER SYSTEM EMPLOYING SAME**

[72] Inventors: **Derek D. Chapman; Leslie G. S. Brooker**, both of Rochester, N.Y.

[73] Assignee: **Eastman Kodak Company**, Rochester, N.Y.

[22] Filed: **May 18, 1970**

[21] Appl. No.: **38,510**

[52] U.S. Cl. .... **96/3, 96/77, 96/29 D,**  
260/240.6

[51] Int. Cl. .... **G03c 7/00, G03c 5/54, G03c 1/40**

[58] Field of Search..... **96/77, 3, 29 D**

[56] **References Cited**

UNITED STATES PATENTS

3,146,102 8/1964 Weyerts et al. .... **96/3**

Primary Examiner—Norman G. Torchin

Assistant Examiner—Alfonso T. Suro Pico

Attorney—W. H. J. Kline, J. R. Frederick and H. E. Cole

[57]

## ABSTRACT

Substituted 1-(dihydroxybenzyl)indocarbocyanine magenta dye developers having the general formula



X-

wherein R represents a hydrogen atom, an alkyl group, or an aryl group, R<sub>1</sub> and R<sub>2</sub> represent alkyl groups or when taken together constitute the number of carbon atoms necessary to form a carbocyclic ring having five, six or seven members and X represents an acid anion, provide improved dye hue and reduced color contamination in diffusion transfer systems.

19 Claims, No Drawings

**MAGENTA DYE DEVELOPER AND TRANSFER SYSTEM  
EMPLOYING SAME**

This invention relates to the art of photography, and, more particularly, to novel dye developers and to their employment in multicolor diffusion transfer systems.

Diffusion transfer color processes have been described in a number of patents, including U.S. Pat. No. 2,983,606, wherein photographic elements containing silver halide emulsion layers and layers containing diffusible dye developers (dyes having a silver halide developing function) are exposed to record the latent image in the silver halide and then treated with an alkaline processing composition which permeates the emulsion layers and layers containing the dye developers which then develop the latent images to silver images. At the same time, oxidation products of the dye developers are formed in situ with the silver images and which are relatively nondiffusing in the colloid vehicle of the layers.

The nondiffusing character of the oxidized dye developers is apparently due, at least in part, to a decrease in solubility in the alkaline processing liquid, and may also be due to a hardening effect of the oxidized developer upon the colloid vehicles of the layers which retards the diffusion of the oxidized dye developers. The residual unoxidized dye developers remaining in the layers in imagewise distribution are transferred by diffusion to a superposed reception element substantially to the exclusion of the silver image and oxidized dye developer to provide a positive dye image.

When an element containing differentially sensitized silver halide emulsion layers is used and subtractively colored dye developers are present in or contiguous to the respective emulsion layers, the dye developers are oxidized and rendered nondiffusing in the developed regions of the layers upon treatment with the processing liquid. The residual dye developer images in the positive regions are transferred by diffusion and in register to the reception element to provide a multicolor reproduction.

Such systems may be used to produce positive images in a single color or in multicolors. In a three-color system, each silver halide emulsion layer has associated therewith a dye developer possessing a spectral absorption range substantially complementary to the predominant sensitivity range of its associated emulsion, i.e., the blue-sensitive silver halide emulsion layer will have a yellow dye developer associated therewith, the green-sensitive silver halide emulsion layer will have a magenta dye developer associated therewith, and the red-sensitive silver halide emulsion layer will have a cyan dye developer associated therewith. The dye developer associated with each silver halide emulsion layer is contained either in a silver halide emulsion layer itself or in a layer contiguous to the silver halide emulsion layer, typically under the silver halide layer with respect to the exposure direction.

As mentioned hereinabove, the magenta dye developer would be normally associated with a green-sensitive silver halide emulsion for use in a three-color system, although it could actually be associated with any light-sensitive silver halide emulsion to obtain e.g., monochrome images, "false color" images etc. The spectral absorption range for a magenta dye developer should be high in the green region of the spectrum and low in the red and blue regions in order to have as little color contamination as possible in the resulting prints. It would be highly desirable to provide a magenta dye developer that is capable of yielding increased absorption in the green region, while at the same time providing less absorption in the red and blue regions as compared with dye developers previously employed.

Accordingly, it is an object of the present invention to provide novel magenta dye developers suitable for use in a multicolor diffusion transfer system that are capable of yielding prints having an improved dye hue and reduced color contamination.

A further object of the present invention is to provide a novel color diffusion transfer system wherein transfer images have increased absorption in the green region of the spectrum

and much less absorption in the red and blue regions when compared to images obtained with prior art magenta dye developers.

These and other objects are achieved in accordance with the present invention with the novel magenta photographic dye developers 1-(dihydroxybenzyl)indocarbocyanine dye developers. It has been found that the dye developers of the present invention possess a spectral absorption range having high absorption in the green region of the spectrum, while at the same time providing very little absorption in the red and blue regions as compared with magenta dye developers of the prior art. Thus, as will be hereinafter illustrated, much less color contamination results if the dye developers of the present invention are employed in a diffusion transfer system than is the case when such known magenta dye developers as 4-isopropoxy-2-[p-β-hydroquinonyethyl]-phenylazo]-1-naphthol described in U.S. Pat. Nos. 3,362,819 and 3,415,644, are employed.

Typical magenta dye developers of the present invention can be characterized by the general formula:



wherein R represents a hydrogen atom, an alkyl group, or an aryl group, R<sub>1</sub> and R<sub>2</sub> represent alkyl groups or when taken together constitute the number of carbon atoms necessary to form a carbocyclic ring having five, six or seven members and X represents an acid anion.

Representative R groups include an alkyl group, preferably a lower alkyl group, i.e., having from one to four carbon atoms in the chain, particularly methyl and ethyl; and an aryl group, e.g., phenyl, etc. Furthermore, substituted alkyl groups are intended to come within the meaning of "alkyl."38 Preferably, the substituted alkyl groups are substituted lower alkyl groups containing from one to four carbon atoms in the chain, such as an aralkyl group, e.g., benzyl, phenethyl, etc., a hydroxyalkyl group, e.g., β-methoxyethyl, etc., a carboxyalkyl group, e.g., β-carboxyethyl, etc., a sulfoalkyl group, e.g., ω-sulfobutyl, etc. Likewise, substituted aralkyl groups are intended to come within the meaning of the term "alkyl." A preferred substituted aralkyl group is a 2,5-dihydroxy benzyl group. Preferably, R represents a methyl group or a 2,5-dihydroxyl group. Preferably, R represents a methyl group or 2,5-dihydroxyl group.

Representative R<sub>1</sub> and R<sub>2</sub> groups include alkyl, preferably lower alkyl having from one to four carbon atoms in the chain, substituted alkyl as defined above, or when taken together a five, six or seven-member carbocyclic ring.

X represents an acid anion, e.g., chloride, bromide, iodide, thiocyanate, sulfamate, perchlorate, p-toluenesulfonate, methyl sulfate, ethyl sulfate, etc.

Examples of dye developers coming within the scope of the above formulae include

- 1,1'-Bis(2,5-dihydroxybenzyl)-3,3;3',3'-di(hexamethylene)-indocarbocyanine perchlorate
- 1,1'-Bis(2,5-dihydroxybenzyl)-3,3;3',3'-di(pentamethylene)-indocarbocyanine perchlorate
- 1,1'-Bis(2,5-dihydroxybenzyl)-3,3;3',3'-di(tetramethylene)-indocarbocyanine perchlorate
- 1-(2,5-Dihydroxybenzyl)-3,3;3',3'-di(pentamethylene)-1'-phenyliindocarbocyanine perchlorate
- 1-(2',5'-Dihydroxybenzyl)-1',3,3;3',3'-pentamethyl-indocarbocyanine perchlorate

1-(2,5-Dihydroxybenzyl)-1'-methyl-3,3;3',3'-di(pentamethylene)indocarbocyanine perchlorate  
 1-(2,5-Dihydroxybenzyl)-3,3-tetramethylene-2-[3-(3,3-pentamethylene-3H-indolyl)allylidene]indoline perchlorate  
 1,1'-Bis(2,5-dihydroxybenzyl)-3,3;3',3'-tetraethylindo-carbocyanine perchlorate  
 1,1'-Bis(2',5'-dihydroxybenzyl)-3,3,3',3'-tetramethyl-indocarbocyanine perchlorate  
 1-(2,5-Dihydroxybenzyl)-1'-propyl-3,3;3',3'-tetramethyl-indocarbocyanine perchlorate  
 1-(2,5-Dihydroxybenzyl)-3,3-dimethyl-2-[3-(3,3-dimethyl-3H-indolyl)allylidene]indoline perchlorate  
 1-(2,5-Dihydroxybenzyl)-3,3-pentamethylene-2-[3-(3,3-pentamethylene-3H-indolyl)allylidene]indoline perchlorate

A particularly preferred embodiment of the present invention involves the provision of a photographic film unit which is adapted to be processed by passing the unit between a pair of juxtaposed pressure-applying members comprising:

- a. a photosensitive element comprising a support having thereon a silver halide emulsion layer having associated therewith a 1-(dihydroxybenzyl) indocarbocyanine dye developer;
- b. a dye image-receiving layer; and
- c. a rupturable container containing an alkaline processing composition,

said rupturable container being adapted to be positioned during processing of said film unit so that a compressive force applied to the container by the pressure applying members will effect a discharge of the container's contents into the film unit.

The dye image-receiving layer of the film unit can be located on a separate support adapted to be superposed on the photosensitive element after exposure thereof. Such image-receiving elements are disclosed, for example, in U.S. Pat. No. 3,362,819. The rupturable container is usually positioned during processing of said film unit so that a compressive force applied to the container by pressure-applying members in a camera will effect a discharge of the container's contents between the image-receiving element and the outermost layer of the photosensitive element. The dye image-receiving layer can also be located integral with the photosensitive element between the support and the lowermost photosensitive silver halide emulsion layer. Such integral receiver-negative photosensitive elements are disclosed, for example, in U.S. Pat. No. 3,415,644 and are useful in camera apparatus of the type disclosed in Belgian Pat. Nos. 718,553 and 718,554. The processing composition for such integral elements wherein the receiver is permanently laminated to the negative contains opacifying agents such as titanium dioxide or carbon black. Barrier layers such as those described in Becker U.S. Pat. No. 3,384,483, may be used to advantage in such integral elements between the various emulsion and dye developer layers.

The color film assembly of the present invention may contain various silver halide emulsion layers disposed in the usual order, i.e., the blue-sensitive silver halide emulsion layer first with respect to the exposure side, followed by the green-sensitive and red-sensitive silver halide emulsion layers. If desired, a yellow dye layer or a Carey Lea silver layer may be present between the blue-sensitive and green-sensitive silver halide emulsion layer for absorbing or filtering clue radiation that may be transmitted through the blue-sensitive layer. If desired, the selectively sensitized silver halide emulsion layers may be disposed in a different order, e.g., the red-sensitive layer first with respect to the exposure side, followed by the green-sensitive and blue-sensitive layers.

Our novel magenta dye developer may be employed in combination with any suitable yellow dye developer and cyan dye developer in a three-color photosensitive element of the invention. Dye developers, i.e., compounds which contain in the same molecule both the chromophoric system of a dye and also a silver halide developing function, and their functioning in color diffusion transfer systems in general are well known in

the art as shown, for example, by U.S. Pat. Nos. 2,983,606; 2,992,106; 3,047,386; 3,076,808; 3,076,820; 3,077,402; 3,126,280; 3,131,061; 3,134,762; 3,134,765; 3,135,604; 3,135,605; 3,135,606; 3,135,734; 3,141,772; and 3,142,565.

5 An alkaline processing or activating composition is conveniently employed in a rupturable container or pod of the film assembly of the present invention. After exposure of the element, the alkaline processing composition is released from the pod to permeate the emulsion layers and initiate development of the latent images contained therein. The dye developers are immobilized in exposed areas as a consequence of the development of the latent images. This immobilization is due at least in part, to a change in the solubility characteristics of the dye developers upon oxidation. In unexposed areas of the emulsion layers, the dye developers remain diffusible and thus provide imagewise distributions of unoxidized dye developer dissolved in the liquid processing composition as a function of the point-to-point degree of exposure of the silver halide emulsion layers. At least part of these imagewise distributions of unoxidized dye developer are transferred, by diffusion, to the image-receiving layer. The image-receiving layer contains materials adapted to mordant or otherwise fix the diffused, unoxidized dye developers.

20 25 Good results are obtained when the dye developers are employed in separate layers contiguous to each silver halide emulsion layer. Such layers can be applied by using coating solutions containing about 0.5 to about 8 percent, by weight, of the dye developer distributed in a hydrophilic film-forming natural material or synthetic polymer such as gelatin, polyvinyl alcohol, etc., which is adapted to be permeated by aqueous alkaline processing composition.

25 In addition to conventional techniques for the direct dispersion of a particulate solid material in a polymeric or colloidal 35 matrix such as ball-milling and the like techniques, the preparation of a dye developer dispersion can also be obtained by dissolving the dye developer in an appropriate solvent or mixture of solvents, dispersing the resultant solution in the polymeric binder, with optional subsequent removal of the 40 solvent or solvents employed. Further details concerning these dispersing techniques and the solvents employed are found, for example, in U.S. Pat. Nos. 2,269,158; 2,322,027; 2,304,939; 2,304,940; 2,801,171, and the like.

45 In a color film unit according to the invention, each silver halide emulsion layer containing a dye developer or having the dye developer present in a contiguous layer may be separated from the other silver halide emulsion layers in the film unit by materials including gelatin, calcium alginate, or any of those 50 disclosed in U.S. Pat. No. 3,384,483, polymeric materials such as polyvinylamides as disclosed in U.S. Pat. No. 3,421,892, or any of those disclosed in U.S. Pat. Nos. 2,992,104; 3,043,692; 3,044,873; 3,061,428; 3,069,263; 3,069,264; 3,121,011; and 3,427,158.

55 Generally speaking, the silver halide emulsion layers in the invention comprise photosensitive silver halide dispersed in gelatin and are about 0.6 to 6 microns in thickness; the dye developers are dispersed in an aqueous alkaline solution-permeable polymeric binder, such as gelatin, as a separate 60 layer about 1 to 7 microns in thickness; and the alkaline solution-permeable polymeric interlayers, e.g., gelatin, are about 1 to 5 microns in thickness. Of course, these thicknesses are approximate only and can be modified according to the product desired.

65 70 75 Use of a polymeric acid layer, as disclosed in U.S. Pat. No. 3,362,819, in the film unit of the present invention will enhance the results obtained. Generally, the polymeric acid layer will effect a reduction in the pH of the image layer from about 13 or 14 to at least 11 and preferably 5-8 within a short time after imbibition. Such polymeric acids reduce the pH of the film unit after development to terminate further dye transfer and thus stabilize the dye image. Such polymeric acids comprise polymers containing acid groups, such as carboxylic acid and sulfonic acid groups, which are capable of forming salts with alkali metals, such as sodium or potassium, or with

organic bases particularly quaternary ammonium bases, such as tetramethyl ammonium hydroxide. The polymers can also contain potentially acid-yielding groups such as anhydrides or lactones or other groups which are capable of reacting with bases to capture and retain them. Generally the most useful polymeric acids contain free carboxyl groups, being insoluble in water in the free acid form and which form water-soluble sodium and/or potassium salts.

The polymeric acid layer is usually about 0.3 to about 1.5 mils in thickness. Although the polymeric acid layer is usually located in the receiver portion of the film unit between the support and the image-receiving layer, it can also be located in the negative portion of the film unit, as disclosed in U.S. Pat. No. 3,362,821.

An inert timing or spacer layer coated over the polymeric acid layer may also be used to "time" or control the pH reduction of the film unit as a function of the rate at which the alkali diffuses through the inert spacer layer. Examples of such timing layers include gelatin, polyvinyl alcohol or any of those disclosed in U.S. Pat. No. 3,455,686. The timing layer is also effective in evening out the various reaction rates over a wide range of temperatures, e.g., premature pH reduction is prevented when imbibition is effected at temperatures above room temperature, for example, at 95° to 100° F. The timing layer is usually about 0.1 to about 0.7 mil in thickness.

The liquid processing composition that may be employed in this invention is, for example, the conventional aqueous solution of an alkaline material, e.g., sodium hydroxide, sodium carbonate or an amine such as diethylamine, preferably possessing a pH in excess of 12. The composition also preferably contains a viscosity-increasing compound such as a high molecular weight polymer, e.g., a water-soluble ether inert to alkaline solutions such as hydroxyethyl cellulose or alkali metal salts of carboxymethyl cellulose such as sodium carboxymethyl cellulose. A concentration of viscosity-increasing compound of about 1 to about 5 percent by weight of the processing composition is preferred which will impart thereto a viscosity of about 100 to about 200,000 c.p.s.

Development of a diffusion transfer element of the invention may also be effected in the presence of an onium compound particularly a quaternary ammonium compound, such as disclosed in U.S. Pat. Nos. 3,146,102; 3,253,915 and 3,173,786.

The silver halide emulsions used with this invention can comprise silver chloride, silver bromide, silver bromoiodide, silver chlorobromoiodide or mixtures thereof. The emulsions may be coarse or fine grain and can be prepared by any of the well-known procedures, e.g., single jet emulsions, double jet emulsions, such as Lippmann emulsions, ammoniacal emulsions, thiocyanate or thioether ripened emulsions such as those described in Nietz et al. U.S. Pat. No. 2,222,264; Illingsworth U.S. Pat. No. 3,320,069; and McBride U.S. Pat. No. 3,271,157. Surface image emulsions can be used or internal image emulsions can be used such as those described in Davey et al. U.S. Pat. No. 2,592,250; Porter et al. U.S. Pat. No. 3,206,313 and Bacon et al. U.S. Pat. No. 3,447,927. The emulsions may be regular grain emulsions such as the type described in Klein and Moisar, *J. Phot. Sci.*, Vol. 12, No. 5, Sept./Oct., 1964 pp. 242-251. If desired mixtures of surface and integral image emulsions can be used as described in Luckey et al. U.S. Pat. No. 2,996,382.

Negative type emulsions can be used or direct positive emulsions can be used such as those described in Leermakers U.S. Pat. No. 2,184,013; Kendall et al. U.S. Pat. No. 2,541,472; Berriman U.S. Pat. No. 3,367,778; Schouwenaars British Pat. No. 723,019; Illingsworth et al. French Pat. No. 1,520,821; Ives U.S. Pat. No. 2,563,785; Knott et al. U.S. Pat. No. 2,456,953 and Land U.S. Pat. No. 2,861,885.

The silver halide emulsions may be unwashed or washed to remove soluble salts. In the latter case the soluble salts may be removed by chill-setting and leaching or the emulsion may be coagulation washed, e.g., by the procedures described in Hewitson et al. U.S. Pat. No. 2,618,556; Yutzy et al. U.S. Pat.

No. 2,614,928; Yackel U.S. Pat. No. 2,565,418; Hart et al. U.S. Pat. No. 3,241,969; and Waller et al. U.S. Pat. No. 2,489,341.

Also, the silver halide emulsions may contain speed increasing compounds such as polyalkylene glycols, cationic surface active agents and thioethers or combinations of these as described in Piper U.S. Pat. No. 2,886,437; Dann et al. U.S. Pat. No. 3,046,134; Carroll et al. U.S. Pat. No. 2,944,900; and Goffe U.S. Pat. No. 3,294,540.

Likewise, the silver halide emulsions can be protected against the production of fog and can be stabilized against loss of sensitivity during keeping. Suitable antifoggants and stabilizers each used alone or in combination include thiazolium salts described in Brooker et al. U.S. Pat. No. 2,131,038 and Allen et al. U.S. Pat. No. 2,694,716; the azaindenes described in Piper U.S. Pat. No. 2,886,437 and Heimbach et al. U.S. Pat. No. 2,444,605; the mercury salts as described in Allen et al. U.S. Pat. No. 2,728,663; the urazoles described in Anderson et al. U.S. Pat. No. 3,287,135; the sulfocatechols described in Kennard et al. U.S. Pat. No. 3,236,652; the oximes described in Carroll et al. British Pat. No. 623,448; nitron; nitroindazoles; the mercaptotetrazoles described in Kendall et al. U.S. Pat. No. 2,403,927; Kennard et al. U.S. Pat. No. 3,266,897 and Luckey et al. U.S. Pat. No. 3,397,987; the polyvalent metal salts described in Jones U.S. Pat. No. 2,839,405; the thiuronium salts described in Herz et al. U.S. Pat. No. 3,220,839; the palladium, platinum and gold salts described in Trivelli et al. U.S. Pat. No. 2,566,263 and Yutzy et al. U.S. Pat. No. 2,597,915.

Any suitable material can be employed as the image-receiving layer in this invention as long as the desired function of mordanting or otherwise fixing the dye developer images will be obtained.

Suitable image-receiving materials include N-methoxymethyl polyhexylmethlene adipamide; partially hydrolyzed polyvinyl acetate; polyvinyl alcohol with or without plasticizers; cellulose acetate; gelatin; and other materials of a similar nature. Polyvinyl alcohol or gelatin containing a dye mordant such as poly-4-vinylpyridine as disclosed in U.S. Pat. No. 3,148,061 can also be employed in the invention with good results. Generally, the image-receiving layer is from about 0.25 to about 0.04 mil in thickness. This thickness, of course, may be modified depending upon the result desired.

The image-receiving layer may also contain ultraviolet absorbing materials to protect the mordanted dye images from fading due to ultraviolet light.

The layers of the photographic element employed and described herein may be coated on a wide variety of supports. Typical supports include cellulose nitrate film, cellulose ester film, poly(vinyl acetal) film, polystyrene film, poly(ethylene terephthalate) film, polycarbonate film and related films or resinous materials, as well as glass, paper, metal and the like. Typically, a flexible support is employed, especially a paper support, which can be partially acetylated or coated with baryta and/or an alpha-olefin polymer, particularly a polymer of an alpha-olefin containing two to ten carbon atoms such as polyethylene, polypropylene, ethylenebutene copolymers and the like.

The photographic elements of this invention can contain incorporated developing agents such as hydroquinones, catechols, aminophenols, 3-pyrazolidones, ascorbic acid and its derivatives, reductones and phenylenediamines. Combinations of developing agents can be employed in the practice of the invention. The developing agents can be in a silver halide emulsion and/or in another suitable location in the photographic element. The developing agents may be added from suitable solvents or in the form of dispersions as described in Yackel U.S. Pat. No. 2,592,368 and Dunn et al. French Pat. No. 1,505,778.

The photographic emulsions and elements described in the practice of the present invention may contain various colloids alone or in combination as vehicles, binding agents and various layers. Suitable hydrophilic materials include both natu-

rally occurring substances such as proteins, for example, gelatin, gelatin derivatives, cellulose derivatives, polysaccharides such as dextran, gum arabic and the like; and synthetic polymeric substances such as water soluble polyvinyl compounds like poly(vinylpyrrolidone), acrylamide polymers and the like.

The described photographic emulsion layers and other layers of the present photographic elements of this invention may also contain alone or in combination with hydrophilic, water permeable colloids, other synthetic polymeric compounds such as dispersed vinyl compounds such as in latex form and particularly those which increase the dimensional stability of the photographic materials. Suitable synthetic polymers include those described, for example, in Nottorf U.S. Pat. No. 3,142,568, issued July 28, 1964; White U.S. Pat. No. 3,193,386, issued July 6, 1965; Houck et al. U.S. Pat. No. 3,062,674, issued Nov. 6, 1962; Houck et al. U.S. Pat. No. 3,220,844, issued Nov. 30, 1965; Ream et al. U.S. Pat. No. 3,287,289, issued Nov. 22, 1966; and Dykstra U.S. Pat. No. 3,411,911, issued Nov. 19, 1968. Particularly effective are those water-insoluble polymers of alkyl acrylates and methacrylates, acrylic acid, sulfoalkyl acrylates or methacrylates, those which have cross-linking sites which facilitate hardening or curing and those having recurring sulfobetaine units as described in Dykstra Canadian Pat. No. 774,054.

The various photographic layers may contain plasticizers and lubricants such as polyalcohols, e.g., glycerin and diols of the type described in Milton et al. U.S. Pat. No. 2,960,404; fatty acids or esters such as those described in Robijns U.S. Pat. No. 2,588,765 and Duane U.S. Pat. No. 3,121,060; and silicone resins such as those described in DuPont British Pat. No. 955,061.

The photographic layers used in the practice of this invention can be coated by various coating procedures including dip coating, air knife coating, curtain coating, or extrusion coating using hoppers of the type described in Beguin U.S. Pat. No. 2,681,294. If desired, two or more layers may be coated simultaneously by the procedures described in Russell U.S. Pat. No. 2,761,791 and Wynn British Pat. No. 837,095. This invention also can be used for silver halide layers coated by vacuum evaporation as described in British Pat. No. 968,453 and LuValle et al. U.S. Pat. No. 3,219,451.

The photographic and other hardenable layers used in the practice of this invention can be hardened by various organic or inorganic hardeners, alone or in combination, such as the aldehydes, and blocked aldehydes, ketones, carboxylic and carbonic acid derivatives, sulfonate esters sulfonyl halides and vinyl sulfonyl ethers, active halogen compounds, epoxy compounds, aziridines, active olefins, isocyanates, carbodiimides, mixed function hardeners and polymeric hardeners such as oxidized polysaccharides like dialdehyde starch and oxygum and the like.

The following examples further illustrate the novel magenta dye developers of the invention:

#### EXAMPLE 1

The compound, 2,3,3-trimethyl-3H-indole, in the amount of 15.9 grams is mixed with 28.7 grams of 2,5-diacetoxybenzyl bromide and the mixture is heated on a steam bath overnight. The 2,5-diacetoxybenzyl bromide is produced in the manner described by D. L. Fields, J. B. Miller and D. D. Reynolds *J. Org. Chem.*, Vol. 29, page 2640 (1964). The crude product is then washed with hot ether. Fifteen grams of the thus-formed diacetoxybenzyl quaternary salt are refluxed in 250 milliliters of ethanol along with 7 grams of 2-(2-acetanilidovinyl)1,3,3-trimethyl-3H indolium iodide and 1.5 grams of triethylamine for a period of 1 hour. The resulting solution is then concentrated on a rotary evaporator and the residue is extracted with hot ether several times. This product is dissolved in 350 milliliters of dimethyl sulfoxide and is heated to a temperature of 45°-50 C. while nitrogen is passed through the solution. Next, 100 milliliters of a 10 percent sodium hydroxide solution are

added and heating is continued for 10 minutes. The reaction mixture is cooled and then acidified with 30 milliliters of concentrated HCl and then poured into one liter of a saturated solution of potassium perchlorate in water. The product is 5 then filtered off and purified by dissolution in acetone and is then precipitated by being poured into the perchlorate solution. A yield of 6 grams of the magenta dye developer, 1-(2',5'-dihydroxybenzyl)-1',3,3,3',3' -pentamethyl-indocarbocyanine perchlorate having a  $\lambda$  max of 547 m $\mu$  is obtained.

10

#### EXAMPLE 2

Thirteen grams of the diacetoxybenzyl quaternary salt prepared in the manner described in Example 1 are admixed with 8 grams of anhydrous sodium acetate and 35 milliliters of diethoxymethyl acetate. The mixture is heated in 30 milliliters of acetic anhydride for a period of 10 minutes. Next, the mixture is cooled and poured into 500 milliliters of a saturated potassium perchlorate solution. One hundred milliliters of ether are added and the mixture is stirred vigorously. After a period of two hours, the solution is filtered. The crude product is hydrolyzed in the manner described in Example 1. A yield of 5 grams of the magenta dye developer, 1,1'-bis(2',5'-dihydroxybenzyl)-3,3',3'-tetramethyl-indocarbocyanine perchlorate is obtained. This material has a  $\lambda$  max of 552 m $\mu$ .

25

#### EXAMPLE 3

Green-sensitive photosensitive elements are prepared by coating a gelatin subbed film support comprising cellulose acetate with suitable hardened gelatin layers as follows:

##### 1. Magenta Dye Developer Layer

The magenta dye developer, 4-isopropoxy-2-[p-( $\beta$ -hydroquinonylethyl)-phenylazo]-1-naphthol, is dissolved in a mixture of cyclohexanone and N-n-butylacetanilide and is dispersed in an aqueous gelatin solution with a sodium alkyl-naphthalene sulfonate dispersing agent. The mixture is passed through a colloid mill several times, coated on the film support and dried to volatilize the cyclohexanone to give a coverage of 64 mg. of the dye developer and 150 mg. of gelatin per square foot of element.

##### 2. Green-Sensitive Emulsion Layer

A green-sensitive silver bromoiodide emulsion is then coated on the magenta dye developer layer at a coverage of 103 mg. of silver and 120 mg. of gelatin per square foot of element.

##### 3. Overcoat Layer

A gelatin overcoat layer is provided on the foregoing layers at a coverage of 150 mg. per square foot of element.

Additional green-sensitive coatings are prepared in the foregoing manner of Example 3 with the exception that the novel magenta dye developers of Examples 1 and 2 are substituted for the magenta dye developer, 4-isopropoxy-2-[p-( $\beta$ -hydroquinonylethyl)-phenylazo]-1-naphthol at coverages, respectively, of 81.5 and 97.5 mg. per square foot of element.

#### EXAMPLE 4

Samples of the film coatings produced in Example 3 are air dried and exposed on an Eastman 1B Sensitometer  $\frac{1}{2}$  inch to a 60 500-watt positive lamp + a 4.08 Corning filter and are processed with a processing solution disposed in a processing pod and having the composition set forth in Table I below:

65

TABLE I

|                                 | Weight (grams) |
|---------------------------------|----------------|
| sodium hydroxide                | 5.54           |
| zinc acetate dihydrate          | 0.19           |
| hydroxyethyl cellulose          | 1.94           |
| sodium thiosulfate pentahydrate | 0.40           |
| benzotriazole                   | 2.32           |
| water to                        | 100.00         |

75

The processing solution is spread between the film and a receiving sheet. The exposed film is processed at a gap of 0.0044 inch for a period of 60 seconds at about 25° C. between a pair of pressure rollers in order to spread the processing solution. The receiving sheet is a cellulose acetate butyrate subbed paper support carrying in the following order:

1. a polymeric acid layer for pH control,
2. a polyvinyl alcohol spacer layer,
3. a mordant layer comprising poly-4-vinyl pyridine and polyvinyl alcohol, and
4. a polyvinyl alcohol protective layer.

## EXAMPLES 5-6

The performance of the magenta dye developers of the present invention is measured by comparing the amount of absorption in the red, green and blue regions of the spectrum of a low, medium and high density area of the transferred image for each coating. The amount of absorption is recorded by a spectrophotometer as optical density. The results are set forth in Table II.

The 610 and 410 m $\mu$  are the red and blue regions of the spectrum, respectively, while the 560 and 535 m $\mu$  is the green region. As can be seen from the foregoing results in Table II, there is more absorption in the green region and less absorption in the red and blue regions for the novel magenta dye developer of the present invention (Example 6) as compared with the prior art dye developer (Example 5). Such results indicate that much of the unwanted absorption in the red and blue regions is eliminated with an increase of green absorption thereby resulting in less color contamination. Similar good results are obtained employing the 1-(2',5'-dihydroxybenzyl)-1',3,3,3',3'-pentamethylene-3H-indole developer of Example 1.

## EXAMPLE 7

The compound, 2-methyl-3,3-pentamethylene-3H-indole, in the amount of 29 grams and 43 grams of 2,5-diacetox-ybenzyl-bromide are dissolved in 100 ml. of acetonitrile and the solution heated under reflux overnight. The acetonitrile is then removed under reduced pressure and the resultant quaternary salt is then treated as in Example 2 to form the indocarbocyanine dye. The crude yield is 60 g. Twenty grams of this product are dissolved in 100 ml. of methanol saturated with HCl and then diluted 1:10 with methanol. The reaction mixture is then stirred overnight and poured into a saturated sodium chloride solution. The product is then filtered off, dried and triturated with acetone. The acetone insoluble fraction is dissolved in 20 ml. of dimethylformamide and poured slowly into a sodium perchlorate solution. A yield of 8 grams of the magenta dye developer 1,1'-bis(2,5-dihydroxybenzyl)-3,3,3',3' having a  $\lambda$  max of 565 m $\mu$  is obtained by filtration having the following structure:



TABLE II

| Example No. | Magenta dye developer                                                                    | Low density area (m $\mu$ ) |       |       |     | Medium density area (m $\mu$ ) |       |       |     | High density area (m $\mu$ ) |       |       |       |
|-------------|------------------------------------------------------------------------------------------|-----------------------------|-------|-------|-----|--------------------------------|-------|-------|-----|------------------------------|-------|-------|-------|
|             |                                                                                          | 610                         | 560*  | 535*  | 410 | 610                            | 560*  | 535*  | 410 | 610                          | 560*  | 535*  | 410   |
| 5.....      | 4-isopropoxy-2-[p-( $\beta$ -hydroquinonyl-ethylphenylazo]-1-naphthol.....               | .30                         | ..... | .71   | .39 | .62                            | ..... | 1.52  | .71 | .58                          | ..... | 1.71  | ..... |
| 6.....      | 1,1'-bis(2',5'-dihydroxybenzyl)-3,3,3',3'-tetramethyl-indocarbo-cyanine perchlorate..... | .18                         | 1.02  | ..... | .36 | .26                            | 1.87  | ..... | .52 | .28                          | 2.00  | ..... | .57   |

\* The reading was taken at the peak.

## EXAMPLE 8

Three grams of the dye developer of Example 7 are dissolved in 25 ml. of dimethyl sulfoxide under nitrogen and heated with 10 ml. of 20 percent sodium hydroxide at 60° C. for two hours. The reaction mixture is chilled in ice and acidified with HCl. The product is filtered off, dissolved in acetone and poured into sodium perchlorate solution. After filtration, a yield of 1.4 grams of the magenta dye developer 1-(2,5-dihydroxybenzyl)-3,3-pentamethylene-2-[3,3-pentamethylene-3H-indolyl]allylideneindoline perchlorate is obtained having the following structure:



## EXAMPLE 9

A control, green-sensitive photosensitive element is prepared by coating a gelatin-subbed cellulose acetate film support with the following layers:

1. Magenta Dye Developer Layer  
The magenta dye developer, 4-isopropoxy-2-[p-( $\beta$ -hydroquinonyl-ethyl)-phenylazo]-1-naphthol is dissolved in a mixture of cyclohexanone and N-nbutylacetanilide and is dispersed in an aqueous gelatin solution with a sodium alkyl-naphthalene sulfonate dispersing agent. The mixture is passed through a colloid mill several times, coated on the film support and dried to volatilize the cyclohexanone to give a coverage of 60 mg. of the dye developer and 150 mg. of gelatin per square foot of element.

2. Green-Sensitive Emulsion Layer  
A green-sensitive silver bromide emulsion is then coated on the magenta dye developer layer at a coverage of 206 mg. of silver and 300 mg. of gelatin per square foot of element.

3. Overcoat Layer  
A gelatin overcoat layer is then provided on the foregoing layers at a coverage of 256 mg. per square foot of element.

An additional green-sensitive element is prepared in the same manner as the control element of this example with the exception that the novel dye developer of Example 7 is substituted for the control dye developer at an equimolar coverage of 102 mg. per square foot of element.

Samples of the two above-described elements are then dipped 5 seconds in a methanol solution containing 4'-methylphenyl hydroquinone and air dried in a vertical position. The elements are then exposed and processed as in Example 4 to give the following print reflectance densities for the

transferred images:

absorb visible light may be included, for instance, ascorbic

| Magenta dye developer                                                                   | Print reflectance densities |       |      |                     |       |      |                      |       |      |
|-----------------------------------------------------------------------------------------|-----------------------------|-------|------|---------------------|-------|------|----------------------|-------|------|
|                                                                                         | Maximum density area        |       |      | Medium density area |       |      | Minimum density area |       |      |
|                                                                                         | Red                         | Green | Blue | Red                 | Green | Blue | Red                  | Green | Blue |
| Control                                                                                 | .26                         | 1.52  | .57  | .20                 | 1.04  | .40  | .10                  | .11   | .13  |
| 1,1'-bis(2,5-dihydroxybenzyl)-3,3,3',3'-di(pentylmethylene)indocarbocyanine perchlorate | .14                         | 1.68  | .16  | .12                 | 1.12  | .16  | .10                  | .12   | .13  |

As can be seen from the foregoing results, an improvement in dye hue is apparent from the decrease in unwanted absorption of the element of the invention as compared to the control, i.e., less density to red and blue light.

**EXAMPLE 10**

Example 9 is repeated but with the novel dye developer of Example 8. Similar results are obtained.

The photographic layers employed in the practice of this invention may contain surfactants such as saponin; anionic compounds such as the alkyl aryl sulfonates described in Baldsiefen U.S. Pat. No. 2,600,831; amphoteric compounds such as those described in Ben-Ezra U.S. Pat. No. 3,133,816; and water soluble adducts of glycidol and an alkyl phenol such as those described in Olin Mathieson British Pat. No. 1,022,878. In addition, the photographic elements may contain matting agents such as starch, titanium dioxide, zinc oxide, silica, polymeric beads including beads of the type described in Jelley et al. U.S. Pat. No. 2,992,101 and Lynn U.S. Pat. No. 2,701,245.

The emulsions used in this invention may be sensitized with chemical sensitizers, such as with reducing agents; sulfur, selenium or tellurium compounds; gold, platinum, or palladium compounds; or combinations of these. Suitable procedures are described in Sheppard et al. U.S. Pat. No. 1,623,499; Waller et al. U.S. Pat. No. 2,399,083; McVeigh U.S. Pat. No. 3,297,447; and Dunn U.S. Pat. No. 3,297,446.

Spectral sensitizing dyes can be used conveniently to confer additional sensitivity to the light-sensitive silver halide emulsion of the multilayer photographic elements of the invention. For instance, additional spectral sensitization can be obtained by treating the emulsion with a solution of a sensitizing dye in an organic solvent or the dye may be added in the form of a dispersion as described in Owens et al. British Pat. No. 1,154,781. For optimum results, the dye may either be added to the emulsion as a final step or at some earlier stage.

Sensitizing dyes useful in sensitizing such emulsions are described, for example, in Brooker et al. U.S. Pat. No. 2,526,632, issued Oct. 24, 1950; Sprague U.S. Pat. No. 2,503,776, issued Apr. 11, 1950; Brooker et al. U.S. Pat No. 2,493,748; and Taber et al. U.S. Pat. No. 3,384,486. Spectral sensitizers which can be used include the cyanines, merocyanines, complex (tri or tetranuclear) merocyanines, complex (tri or tetranuclear) cyanines, holopolar cyanines, styryls, hemicyanines (e.g., enamine hemicyanines), oxonols and hemioxonols. Dyes of the cyanine classes may contain such basic nuclei as the thiazolines, oxazolines, pyrrolines, pyridines, oxazoles, thiazoles, selenazoles and imidazoles. Such nuclei may contain alkyl, alkylene, hydroxyalkyl, sulfoalkyl, carboxyalkyl, aminoalkyl and enamine groups and may be fused to carbocyclic or heterocyclic ring systems either unsubstituted or substituted with halogen, phenyl, alkyl, haloalkyl, cyano, or alkoxy groups. The dyes may be symmetrical or unsymmetrical and may contain alkyl, phenyl, enamine or heterocyclic substituents on the methine or polymethine chain. The merocyanine dyes may contain the basic nuclei mentioned above as well as acid nuclei such as thiohydantoins, rhodanines, oxazolidenediones, thiazolidenediones, barbituric acids, thiazolineones, and malononitrile. These acid nuclei may be substituted with alkyl, alkylene, phenyl, carboxyalkyl, sulfoalkyl, hydroxyalkyl, alkoxyalkyl, alkylamino groups, or heterocyclic nuclei. Combinations of these dyes may be used, if desired. In addition, supersensitizing addenda which do not

acid derivatives, azaindenes, cadmium salts, and organic sulfonic acids as described in McFall et al. U.S. Pat. No. 2,933,390 and Jones et al. U.S. Pat. No. 2,937,089.

The various layers, including the photographic layers, employed in the practice of this invention can contain light absorbing materials and filter dyes such as those described in Sawdey U.S. Pat. No. 3,253,921; Gaspar U.S. Pat. No. 2,274,782; Silberstein et al. U.S. Pat. No. 2,527,583 and Van-Campen U.S. Pat. No. 2,956,879. If desired, the dyes can be mordanted, for example, as described in Jones et al. U.S. Pat. No. 3,282,699.

No. 3,282,099.  
The photographic elements used in this invention may contain brightening agents including stilbenes, triazines, oxazoles and coumarin brightening agents. Water soluble brightening agents may be used such as those described in Albers et al. German Pat. No. 972,067 and McFall et al. U.S. Pat. No. 2,933,390 or dispersions of brighteners may be used such as those described in Jansen German Pat. No. 1,150,274, Oetiker et al. U.S. Pat. No. 3,406,070 and Heidke French Pat. No. 1,530,244.

The sensitizing dyes and other addenda used in the practice of this invention may be added from water solutions or suitable organic solvent solutions may be used. The compounds can be added using various procedures including those described in Collins et al. U.S. Pat. No. 2,912,343; McCrossen et al. U.S. Pat. No. 3,342,605; Audran U.S. Pat. No. 2,996,287 and Johnson et al. U.S. Pat. No. 3,425,835.

The invention has been described with particular reference to certain preferred embodiments thereof, but it will be understood that variations and modifications can be effected within the spirit and scope of the invention.

We claim

1. A photosensitive element comprising a support coated with a silver halide emulsion layer having associated therewith a 1-(dihydroxybenzyl)indocarbocyanine dye developer.
  2. A photosensitive element comprising a support having thereon the following layers in sequence:
    - a cyan dye developer layer,
    - a red-sensitive silver halide emulsion layer,
    - c. a magenta dye developer layer comprising a 1-(dihydroxybenzyl)indocarbocyanine,
    - d. a green-sensitive silver halide emulsion layer,
    - e. a yellow dye developer layer, and
    - f. a blue-sensitive silver halide emulsion layer.
  3. The photosensitive element of claim 2 wherein said magenta dye developer has the formula:



wherein R represents a hydrogen atom, an alkyl group or an aryl group, R<sub>1</sub> and R<sub>2</sub> represent alkyl groups or when taken together constitute the number of carbon atoms necessary to form a carbocyclic ring having five, six or seven members and X represents an acid anion.

4. The photosensitive element of claim 3 wherein R represents a methyl group or a 2,5-dihydroxy benzyl group, each R<sub>1</sub> is a methyl group and each R<sub>2</sub> is a methyl group.

5. The photosensitive element of claim 3 wherein R is hydrogen or a 2,5-dihydroxy benzyl group and each R<sub>1</sub> and R<sub>2</sub> taken together form a six-member carbocyclic ring.

6. A photographic film unit which is adapted to be processed by passing said unit between a pair of juxtaposed pressure-applying members comprising:

- a. a photosensitive element comprising a support having thereon a silver halide emulsion layer having associated therewith a 1-(dihydroxybenzyl)indocarbocyanine dye developer;
- b. a dye image-receiving layer; and
- c. a rupturable container containing an alkaline processing composition;

said rupturable container being adapted to be positioned during processing of said film unit so that a compressive force applied to said container by said pressure-applying members will effect a discharge of the container's contents within said film unit.

7. The film unit of claim 6 wherein said dye image-receiving layer is located in said photosensitive element between said support and said silver halide emulsion layer.

8. The film unit of claim 6 wherein said photosensitive element comprises a support having thereon the following layers in sequence:

- a. a cyan dye developer layer,
- b. a red-sensitive silver halide emulsion layer,
- c. a magenta dye developer layer comprising a 1-(dihydroxybenzyl)indocarbocyanine,
- d. a green-sensitive silver halide emulsion layer,
- e. a yellow dye developer layer, and
- f. a blue-sensitive silver halide emulsion layer.

9. The film unit of claim 8 wherein said dye image-receiving layer is coated on a separate support and is adapted to be superposed on said photosensitive element after exposure thereof.

10. The film unit of claim 9 wherein said rupturable container is so positioned during processing of said film unit that a compressive force applied to said container by said pressure-applying members will effect a discharge of the container's contents between said dye image-receiving layer and the outermost layer of said photosensitive element.

11. The film unit of claim 10 wherein said magenta dye developer has the formula:



wherein R represents a hydrogen atom, an alkyl group or an aryl group, R<sub>1</sub> and R<sub>2</sub> represent alkyl groups or when taken together constitute the number of carbon atoms necessary to form a carbocyclic ring having five, six or seven members and X represents an acid anion.

12. The film unit of claim 11 wherein R represents a methyl group or a 2,5-dihydroxy benzyl group, each R<sub>1</sub> is a methyl group and each R<sub>2</sub> is a methyl group.

13. The film unit of claim 11 wherein R is hydrogen or a 2,5-dihydroxy benzyl group and each R<sub>1</sub> and R<sub>2</sub> taken together form a six-member carbocyclic ring.

14. A process for producing a photographic transfer image comprising:

- a. imagewise exposing a photosensitive element comprising a support having thereon a silver halide emulsion layer

having associated therewith a 1-(dihydroxybenzyl)indocarbocyanine dye developer;

- b. treating said photosensitive element with an alkaline processing composition to effect development of said exposed silver halide emulsion layer;
- c. forming an imagewise distribution of diffusible dye developer as a function of said imagewise exposure of said silver halide emulsion layer; and
- d. at least a portion of said imagewise distribution of diffusible dye developer diffusing to a dye image-receiving layer.

15. The process of claim 14 wherein said treatment step b) is effected by:

- a. superposing over the layer outermost from the support of said photosensitive element said dye image-receiving layer coated on a support;
- b. positioning a rupturable container containing said alkaline processing composition between said exposed photosensitive element and said dye image-receiving layer; and
- c. applying a compressive force to said container to effect a discharge of the container's contents between said outermost layer of said exposed photosensitive element and said dye image-receiving layer.

16. A process for producing a photographic transfer image in color comprising:

- a. imagewise exposing a photosensitive element comprising a support having thereon the following layers in sequence:
  - a. a cyan dye developer layer,
  - b. a red-sensitive silver halide emulsion layer,
  - c. a magenta dye developer layer comprising a 1-(dihydroxybenzyl)indocarbocyanine,
  - d. a green-sensitive silver halide emulsion layer,
  - e. a yellow dye developer layer, and
  - f. a blue-sensitive silver halide emulsion layer,
- b. superposing over the layer outermost from the support of said photosensitive element a dye image-receiving layer coated on a support;
- c. positioning a rupturable container containing an alkaline processing composition between said exposed photosensitive element and said dye image-receiving layer;
- d. applying a compressive force to said container to effect a discharge of the container's contents between said outermost layer of said exposed photosensitive element and said dye image-receiving layer;
- e. thereby effecting development of each of said exposed silver halide emulsion layers;
- f. forming an imagewise distribution of diffusible dye developer as a function of said imagewise exposure of each of said silver halide emulsion layers; and
- g. at least a portion of each of said imagewise distributions of diffusible dye developer diffusing to said dye image-receiving layer.

17. The process of claim 16 wherein said magenta dye developer has the formula:



wherein R represents a hydrogen atom, an alkyl group or an aryl group, R<sub>1</sub> and R<sub>2</sub> represent alkyl groups or when taken together constitute the number of carbon atoms necessary to form a carbocyclic ring having five, six or seven members and X represents an acid anion.

**15**

18. The process of claim 17 wherein R represents a methyl group or a 2,5-dihydroxy benzyl group, each R<sub>1</sub> is a methyl group and each R<sub>2</sub> is a methyl group.

19. The process of claim 17 wherein R is hydrogen or a 2,5-

**16**

dihydroxy benzyl group and each R<sub>1</sub> and R<sub>2</sub> taken together form a six-member carbocyclic ring.

\* \* \* \* \*

5

10

15

20

25

30

35

40

45

50

55

60

65

70

75